

Nov. 21, 1950

E. F. LOWRY ET AL

2,530,394

ELECTRODE COATING FOR DISCHARGE DEVICES

Filed June 5, 1947



*Erwin F. Lowry  
Eric L. Mager  
Gerald W. Keilholtz*

INVENTORS

BY *Lorraine Boone*

ATTORNEY

## UNITED STATES PATENT OFFICE

2,530,394

## ELECTRODE COATING FOR DISCHARGE DEVICES

Erwin F. Lowry, Lynn, Eric L. Mager, Peabody,  
and Gerald W. Keilholtz, Lynn, Mass., assignors  
to Sylvania Electric Products, Inc., Salem,  
Mass., a corporation of Massachusetts

Application June 5, 1947, Serial No. 752,698

20 Claims. (Cl. 176—126)

1

This invention relates to electric gaseous discharge devices and more particularly to fluorescent lamps and the composition of the coating material with which the lamp electrodes are provided.

An object of this invention is to provide an efficient electrode coating for electric gaseous discharge devices.

Another object is to provide an electrode coating which will effect a lengthening of the life of the device in which the electrode is employed.

A further object is to provide an electrode coating which will enhance the lumens per watt maintenance of the device in which the electrode is employed.

A further object is to provide a new coating composition for fluorescent lamp electrodes.

A further object is to provide a coating composition for fluorescent lamp electrodes which will have a beneficial effect in reducing various types and forms of discoloration which sometimes develop on the wall of the lamp during life.

Further objects, advantages, and features will be apparent from the following specification when read in conjunction with the accompanying drawing in which the figure is a view of a fluorescent lamp partly in section.

In the drawing a light-transmitting tubular envelope 1, of glass or the like, is coated on its inner wall with a fluorescent material 2 such as tungstates or silicates, for example, magnesium tungstate or zinc beryllium silicate. The envelope 2 is provided, at each end, with a stem 3, through which lead wires 4 and 5 extend.

A tungsten wire filamentary electrode 6, coated with electron-emissive material, is mounted on the inner ends of the lead wires 4 and 5. The outer ends of the lead wires 4 and 5 are connected to pins 7 and 8 of a base 9 which is secured to the ends of the envelope 1. The sealed envelope is provided with a filling of inert gas at a low pressure, such as argon at about 3 mm., and a small quantity of mercury 11 to provide mercury vapor. The lamp is ordinarily operated at a mercury vapor pressure of between 1 to 20 microns.

In the manufacture of electric gaseous discharge devices, and more particularly in the manufacture of fluorescent lamps of the "hot cathode" type, i. e., those in which the electrodes comprise a coiled filament of tungsten wire, such as that shown in U. S. Patent 2,258,158, for example, the electrodes are usually provided with a coating of an electron-emissive material. As in the patent mentioned above, the electrode wire can be wound into a minor coil and the latter itself then wound into a major coil to form a coiled-coil with the electron-emissive coating material filling the space within the minor coil only. In the case of a fluorescent lamp electrode, the electron emissive material usually com-

2

prises an oxide of one or more of the alkaline earth metals. For convenience, the alkaline earth metals are usually applied in the form of a carbonate which breaks down to the oxide when the lamp is processed.

Many times, during the life of a fluorescent lamp, discoloration of various types and forms appears on the wall of the lamp near the ends thereof and in proximity to the electrodes. It is an object of this invention to reduce the frequency of occurrence and intensity of these discolorations. Three types of discolorations which are affected by the new electrode coating composition of our invention are, electrode spots, end bands, and multiples.

Electrode spots are dark gray or black spots which appear on the inner wall of the lamp near the ends thereof, and are usually found approximately opposite the electrodes. End bands are rings of discoloration, usually light yellow, brownish or black, which usually extend completely around the periphery of the inner wall of the lamp. End bands are usually defined by a sharp edge on the side near the electrode and a diffused edge on the side near the longitudinal center of the lamp. End bands are usually round forward of the electrodes with the sharp edge located opposite the end of the positive column discharge. Multiples are narrow crescents of discoloration, usually light yellow, brownish, or black, which appear near the ends of the lamp on both sides of the electrodes, i. e., on the base side of the electrode as well as the side near the longitudinal center of the lamp.

We have found that the addition of zirconium dioxide in proper amounts to the basic electron emissive material with which the electrodes are coated will not only reduce the frequency of appearance and intensity of the above described discolorations but will also extend the useful life of the lamp and increase the lumens per watt maintenance during life.

In the preparation of the basic electron emissive material we prefer to use a triple carbonate, of the alkaline earth metals, i. e.,  $\text{SrCO}_3$ ,  $\text{BaCO}_3$ , and  $\text{CaCO}_3$ . However, a double or single carbonate may be employed without departing from the spirit of our invention. The carbonates may be prepared in any suitable manner well known in the art. In the preparation of the triple carbonate we have found the following composition to be very satisfactory: about 35%  $\text{SrCO}_3$ , about 58%  $\text{BaCO}_3$ , and about 7%  $\text{CaCO}_3$ , all percentages being by weight. However, these percentages may be varied widely and, as mentioned above, a double or single carbonate may be used without departing from the spirit of our invention.

A small quantity of zirconium dioxide is added to the alkaline earth carbonates. The quantity

of  $ZrO_3$  may vary from between about 1% to about 20% by weight based on the total weight of the carbonates to which it is added. We have found that the addition of about 5% by weight based on the weight of the carbonates gives exceptionally good results. If less than 1% is used, we have found no appreciable improvement is effected. On the other hand, if more than 20%  $ZrO_2$  is added, the frequency of occurrence and intensity of discoloration increases and it becomes more difficult to start the lamps at normal starting voltages. Tables I, II and III below show the extent to which the addition of small quantities of  $ZrO_2$  to the electrode coating material effects a reduction in discoloration, an increase in the L. P. W. late in life, and a lengthening of the life of the lamps. The lamps on which these tests were made were exactly the same as those manufactured on standard production runs, with the sole exception that some  $ZrO_2$  was added to the electrode coating material of some of the lamps. The same fluorescent material, quantity of mercury, amount of gas filling etc., was used. The lamps were processed on the same exhaust machine at the same time. Other tests have shown results similar to those tabulated below.

Table I shows, in percent, the number of lamps, of the hundreds which were checked, which were free of any discoloration at 100, 300, and 500 hours of operation. Tests A, B and C represent 40 watt fluorescent lamps in which the electrode coating contained no  $ZrO_2$ . In Test D, about 5%  $ZrO_2$  was added to the electrode coating material.

Table I

| Test.....                        | A   |     |     | B   |     |     | C   |     |     | D   |     |     |
|----------------------------------|-----|-----|-----|-----|-----|-----|-----|-----|-----|-----|-----|-----|
| Hours.....                       | 100 | 300 | 500 | 100 | 300 | 500 | 100 | 300 | 500 | 100 | 300 | 500 |
| Per Cent<br>C lean<br>Lamps..... | 80  | 46  | 26  | 83  | 63  | 33  | 75  | 52  | 43  | 93  | 90  | 87  |

Table II shows the average L. P. W. of lamps late in life. In this test, five lamps had no  $ZrO_2$  in the electrode coating, five lamps had 5%  $ZrO_2$  in the electrode coating and five lamps had 10%  $ZrO_2$  in the electrode coating.

Table II

|                 | 0% $ZrO_2$<br>L. P. W. | 5% $ZrO_2$<br>L. P. W. | 10% $ZrO_2$<br>L. P. W. |
|-----------------|------------------------|------------------------|-------------------------|
| 2544 hours..... | 40.8                   | 41.6                   | 41.6                    |
| 4040 hours..... | 38.8                   | 40.0                   | 40.4                    |
| 6131 hours..... |                        | 38.8                   | 37.8                    |

Table III shows the time at which the lamps of Table II failed.

Table III

| 0% $ZrO_2$ | 5% $ZrO_2$                         | 10% $ZrO_2$ |
|------------|------------------------------------|-------------|
| Hours      |                                    |             |
| 3,978      | No failures up to 7,068 hours..... |             |
| 4,116      |                                    | 5,989       |
| 4,116      |                                    | 6,503       |
| 4,422      |                                    | 6,645       |
| 4,742      |                                    |             |

The above tables clearly illustrate the several beneficial effects which may be obtained by adding a small quantity of zirconium dioxide to the electrode coating material. Table I indicates that not only is there a decrease in the discoloration of lamps very early in life, i. e. at 100 hours, but the rate at which discoloration begins to appear at 300 and 500 hours for example, is extremely

low when compared to the rapid appearance of discoloration at 300 and 500 hours in lamps in which the electrode coating contains no zirconium dioxide. The beneficial effect which the addition of zirconium dioxide to the electrode coating has on the L. P. W. of the lamps late in life is illustrated in Table II. For example, lamps with no  $ZrO_2$  in the electrode coating read 38.8 L. P. W. at 4040 hours whereas this same reading was obtained at 6131 hours with lamps having 5%  $ZrO_2$  in the electrode coating material. The effect which the addition of small quantities of  $ZrO_2$  has on the life as illustrated in Table III, is tremendous. The average life of the lamps with 15 no  $ZrO_2$  in the electrode coating was about 4200-4300 hours; the first failure of the lamps with 10%  $ZrO_2$  in the electrode coating did not occur until almost 6000 hours; and the 7000 hour mark has been passed without a single failure 20 among the five lamps with 5%  $ZrO_2$  in the electrode coating material.

As mentioned above, the tungsten wire filamentary electrodes of fluorescent lamps are usually provided with an electron-emissive coating 25 of the oxide of one or more of the alkaline earth metals. For convenience this material is usually applied to the electrodes in the form of a carbonate which is later broken down to give the oxide. For this reason, therefore, the proportions given above with reference to the amount 30 of  $ZrO_2$  which is added (1% to 20%) are based on the weight of the mixed carbonates to which the  $ZrO_2$  is added. This is equivalent to a percentage range of from slightly less than 1% to 35 about 17% based upon the total weight of the batch materials after mixing and a percentage range of from slightly more than 1% to about 22% of the total weight of the mixed oxides to which the batch is subsequently converted during 40 lamp processing. The preferential amount of  $ZrO_2$  which has been described as about 5% by weight based on the weight of the mixed carbonates is slightly less than 5% by weight of the total batch after mixing and is slightly more than 6% of the total weight of the mixed oxides finally obtained. The 10%  $ZrO_2$  in Table III is based on the total weight of the mixed carbonates to which the zirconium dioxide is added. This is equivalent to about 11% of the final weight of the 45 mixed oxide, the carbonate being converted to oxides during the lamp processing, as previously explained.

#### What we claim is:

1. A coating material for electric gaseous discharge device electrodes comprising at least one oxide of an alkaline earth metal and a quantity of zirconium dioxide equal to about 6% by weight of the total weight of all the oxides.

2. A coating material for electric gaseous discharge device electrodes comprising oxides of at least two of the alkaline earth metals and a quantity of zirconium dioxide equal to about 6% by weight of the total weight of all the oxides.

3. A coating material for electric gaseous discharge device electrodes comprising oxides of barium, strontium and calcium, and a quantity of zirconium dioxide equal to about 6% by weight of the total weight of all the oxides.

4. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, 70 said coating comprising oxides of barium, strontium

num and calcium and a quantity of zirconium dioxide in an amount more than about 1% but not more than 11% by weight of the total weight of all the oxides.

5. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating comprising at least one oxide of an alkaline earth metal and a quantity of zirconium dioxide equal to about 6% by weight of the total weight of all the oxides.

6. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating comprising oxides of at least two of the alkaline earth metals and a quantity of zirconium dioxide equal to about 6% by weight of the total weight of all the oxides.

7. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating comprising oxides of barium, strontium and calcium and a quantity of zirconium dioxide equal to about 6% by weight of the total weight of all the oxides.

8. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating comprising at least one oxide of an alkaline earth metal and a quantity of zirconium dioxide in an amount more than about 1% but not more than 11% by weight of the total weight of all the oxides.

9. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating comprising oxides of at least two of the alkaline earth metals and a quantity of zirconium dioxide in an amount more than about 1% but not more than 11% by weight of the total weight of all the oxides.

10. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating consisting essentially of at least one oxide of an alkaline earth metal and a quantity of zirconium dioxide in an amount more than about 1% but not more than 11% by weight of the total weight of all the oxides.

11. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating consisting essentially of oxides of at least two of the alkaline earth metals

and a quantity of zirconium dioxide in an amount more than about 1% but not more than 11% by weight of the total weight of all the oxides.

12. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating consisting essentially of oxides of barium, strontium and calcium and a quantity of zirconium dioxide in an amount more than about 1% but not more than 11% by weight of the total weight of all the oxides.

13. A low-pressure fluorescent lamp comprising an elongated sealed light-transmitting envelope, a coating of fluorescent material on the inner wall of said envelope, a quantity of mercury in said envelope, a filamentary electrode of coiled tungsten wire at each end of said envelope, and an electron-emissive material carried by said electrode and comprising at least one oxide of an alkaline earth metal and a quantity of zirconium dioxide in an amount between about 1% and 11% by weight of the total weight of all the oxides carried by said electrode.

14. A fluorescent lamp comprising a sealed light-transmitting envelope, a coating of fluorescent material on the inner wall of said envelope, a quantity of mercury of said envelope, a filling of inert gas in said envelope, filamentary electrodes in said envelope, and a coating on said electrodes, said coating comprising at least one oxide of an alkaline earth metal and a quantity of zirconium dioxide in a critical amount between zero percent and eleven percent of the total weight of all the oxides, and corresponding to an amount therebetween giving substantially maximum cathode life within said range.

15. A fluorescent lamp comprising a sealed light-transmitting envelope, a coating of fluorescent material on the inner wall of said envelope, a quantity of mercury in said envelope, a filling of inert gas in said envelope, filamentary electrodes in said envelope, and a coating on said electrodes, said coating consisting essentially of oxides and including at least one oxide of an alkaline earth metal and a quantity of zirconium dioxide in a critical amount, between zero percent and eleven percent of the total weight of all the oxides, and corresponding to an amount therebetween giving substantially maximum cathode life within said range.

16. A fluorescent lamp comprising a sealed light-transmitting envelope, a coating of fluorescent material on the inner wall of said envelope, a quantity of mercury in said envelope, a filling of inert gas in said envelope, a filamentary electrode of coiled tungsten wire at each end of said envelope, and an electron-emissive material carried by said electrode and consisting essentially of oxides and including at least one oxide of an alkaline earth metal and a quantity of zirconium dioxide in a critical amount, between zero percent and eleven percent of the total weight of all the oxides, and corresponding to an amount therebetween giving substantially maximum cathode life within said range.

17. A fluorescent lamp comprising a sealed elongated light-transmitting tubular envelope, a coating of fluorescent material on the inner wall of said envelope, a quantity of mercury in said envelope, a filling of inert gas at low pressure within said envelope, a filamentary electrode at each end of said envelope and wound into a minor

coil with the latter wound into a major coil to form a coiled-coil, and an electron-emissive coating material filling the space within said minor coil only and comprising at least one oxide of an alkaline earth metal and a quantity of zirconium dioxide in a critical amount between zero and eleven percent of the total weight of all the oxides and corresponding to an amount there-between giving substantially maximum cathode life within said range.

18. The combination of claim 14, in which the oxide of the alkaline earth metal is a reduced carbonate.

19. The combination of claim 13, in which the filamentary electrode of coiled tungsten wire is wound into a minor coil with the latter wound into a major coil to form a coiled-coil, and the electron emissive material fills the space within said minor coil only.

20. The combination of claim 13, in which the oxide of the alkaline earth metal is a reduced carbonate.

ERWIN F. LOWRY.

ERIC L. MAGER.

GERALD W. KEILHOLTZ.

#### REFERENCES CITED

The following references are of record in the 10 file of this patent:

#### UNITED STATES PATENTS

| Number    | Name           | Date           |
|-----------|----------------|----------------|
| 1,821,359 | Reerink et al. | Sept. 1, 1931  |
| 1,823,984 | Nicolson       | Sept. 22, 1931 |
| 1,903,144 | Spanner        | Mar. 28, 1933  |
| 2,238,595 | McNall         | Apr. 15, 1941  |
| 2,249,672 | Spanner        | July 15, 1941  |